

March 26, 1968

R. D. PITTMAN

3,375,179

METHOD OF ANODIZING BERYLLIUM AND PRODUCT THEREOF

Filed Oct. 29, 1964



INVENTOR:  
Richard D. Pittman



Attorney

## 1

3,375,179

METHOD OF ANODIZING BERYLLIUM AND  
PRODUCT THEREOF

Richard D. Pittman, Burbank, Calif., assignor to Litton Systems, Inc., Beverly Hills, Calif.  
Filed Oct. 29, 1964, Ser. No. 407,454  
4 Claims. (Cl. 204—32)

This invention relates to the treatment of metals and, more particularly, to methods, products, and processes for producing anodic films on beryllium metal.

It has long been known that beryllium would be a very valuable metal if it could be properly worked and handled in various manufacturing processes. The metal is especially light and strong; it has the most favorable strength-to-weight ratio of all light metals. Its conductivity is approximately forty percent that of copper. Beryllium melts at 1285° C., a temperature higher than the melting point of copper. It has an unusually high modulus of elasticity. It has substantially no tendency to warp, exhibits very little change in dimensions with temperature, is an especially good thermal conductor, and has various other attributes which are desirable. Such characteristics make beryllium especially useful in situations where weight, strength, and resistance to dimensional change are important, e.g., in precision instruments.

Until recently, however, the manufacturing technology relating to beryllium has been substantially limited. The limited technology has confined the use of the metal to particular situations. For example, beryllium has a very low atomic number and a low absorption characteristic which make it penetrable by X-rays so the pure metal has been used as "windows" in X-ray tubes for selective filtration of "soft" X-rays. It has also been used in atomic reactors. A number of useful alloys have been formed with copper, aluminum, nickel, gold, and iron. In general, these alloys are quite hard; for example, beryllium-copper is the hardest copper-based alloy known.

These few areas clearly do not make full use of beryllium's valuable properties. The main problem in further utilizing beryllium has been that its crystalline structure is such that it, essentially, cannot be worked by conventional methods. For example, the crystals normally formed on solidifying from the cold state are so large that machining, cold rolling, and other processes were impractical. However, the advent of powder metallurgy (see, The Metal Beryllium, White & Burke, published 1955, by the American Society for Metals) allowed the revision of the crystalline structure of beryllium in a manner such that it may now be practically machined and worked. As a matter of fact, one of beryllium's attractive features is the ease with which it may now be machined.

A second problem has been that beryllium oxide, a normal source and by-product of beryllium, has been thought to be a health hazard like the oxide of lead. However, by practicing well understood precautions, the hazard to health has been substantially eliminated.

Having thus solved the problem of machining beryllium and having determined that the hazard offered to health might be circumvented, it would seem that the way stood open to exploit the metal to its fullest. However, there the technology stopped. Whereas other materials such as steel, aluminum, and the like may be coated and otherwise treated in manners such as to render them corrosion resistant, attractive, heat emissive, and bondable, the methods for so treating beryllium having been severely limited. To some extent this is due to its inherent corrosion resistance; that is, since the metal displayed the characteristic, little study has been directed toward its improvement. This property though useful, is not sufficient for many situations, however. Electroplating processes

## 2

have been used for coating beryllium with a metal. However, these coatings are conductive and only as corrosion resistant as the particular metal. At elevated temperatures, no good non-metallic protective coating exists. The problem is complicated by the tendency of beryllium to form hard-brITTLE diffusion phases with the coatings. Thus, though aluminum may be anodized to form a protective coating of aluminum oxide, it has heretofore been possible to produce only an uneven black coating on beryllium. The coating produced is generally so slick that bonding with commercial epoxy adhesives is practically impossible. It is not sufficiently dielectric unless made so thick as to radically affect dimensions. The only really usable property of the coating is its black color which enables it to emit a substantial amount of heat when used in heat-sensitive, temperature-controlled situations. A number of other coatings have been suggested; but, in general, these coatings attack the beryllium metal, changing the dimensions and weakening the structure so that their use is drastically limited.

Thus, the prior art has been unable to provide for beryllium a heat emissive, dielectric, integral, bondable coating the dimensions of which may be exactly controlled. The use of beryllium has suffered drastically from this lack. Some researchers have alloyed beryllium with other metals in order to obtain such a coating thereby diluting the effects of beryllium's desirable properties. Others have used mixtures of other materials with beryllium to the same effect. Therefore, attempts to anodize have continued.

In attempting to provide a black, dielectric protective coating for beryllium metal, many known commercial anodizing processes for beryllium and other metals were evaluated. In general, the commercial coatings, like aluminum anodizing coatings, build up to cover the base metal increasing its dimensions. Many of the processes were found to produce a conductive coating when the coatings were applied to a reasonable thickness, one which did not distort dimensions. Non-conductivity, it should be noted, affords protection against galvanic corrosion; it also extends the use of beryllium in electrical instruments. Most of the commercial coatings had to be made so thick to obtain the desired dielectric properties that the dimensions of the parts were appreciably changed. Thus, design allowances for dimensional changes were required.

Many of the commercial processes produced coatings with other undesirable features. For example, none of the coatings had surfaces which facilitated epoxy bonding to other materials. Many afforded little protection from corrosion and abrasion. All in all, no satisfactory coating was found in the prior art.

To this end, extensive experiments were conducted to devise a new technique for coating beryllium metal in accordance with the above-stated criteria.

I have now discovered a unique method for providing beryllium with a surface coating having characteristics which are almost selectable at will. A preferred form of the coating is hard, extremely heat conductive, of selectable color, and exhibits excellent dielectric properties. My method is especially useful because the coating may be formed evenly and consistently to provide the desired dimensions over almost any texture of surface of the beryllium metal. Thus, a rough-textured beryllium surface, a smooth shiny beryllium surface, a striated beryllium surface, or substantially any other beryllium surface may be prepared. Further, the thickness may be limited so that it does not appreciably affect dimensions of the coated part yet provides the desired characteristics. Bonding to the coating by commercial methods has proven quite effective. In addition, the method is very inexpensive, requires a short time, is substantially insensitive to the

looseness of controls practiced, and has many other desirable features.

It is therefore a primary object of my invention to cover beryllium with a hard integral layer of material having a selectable dielectric constant, a selectable coloration, and a consistent selectable thickness.

Yet another object of my invention, in a primary sense, is to anodize beryllium metal.

Another object of my invention is to cover beryllium metal evenly without changing its dimensions materially.

An additional object of my invention is to provide coatings for beryllium metal by easily controlled processes.

It is another object of my invention to anodize beryllium to form a hard, heat-conductive, dielectric coating of even thickness thereon.

An additional object of my invention is to anodize beryllium with a coating of material having a thickness which may be accurately controlled to minimum dimensions.

Yet another object of my invention is to anodize beryllium with coatings to which other materials may be easily bonded by commercial methods.

In realizing the above objects, I have devised processes which are especially inexpensive and require a minimum of control. For example, in a preferred process the material may be cleaned by substantially any method desired. Thus, the surface of the metal may be prepared in a manner such that it is dull, bright, or has almost any other desired characteristic. The coating which forms may be made so thin that the final surface is substantially identical to the original and exhibits its characteristics. After surface preparation, the part to be coated is connected to a positive source of DC potential; the negative terminal of the DC source is connected to an inert cathode material, e.g., the container holding the coating bath. The part is immersed in the coating solution; and the circuit is energized, either before or after the immersion. Depending on the time, temperature, and material of which the bath is composed, a coating is formed on the beryllium having a particular color, a particular thickness, and others of the aforementioned characteristics, as desired.

The process, of course, depends upon the bath. I have determined that the most useful bath from the standpoint of characteristics includes sodium borate and sodium hydroxide proportioned to provide an excess of hydroxyl ions. When energized at a low initial voltage for periods greater than fifteen minutes, the desired black, bondable, dielectric coating is produced.

It should be especially noted, before proceeding to a more specific description of my processes, that the baths which I use for the anodic coatings for beryllium metal are varied yet fall within substantially a class of solutions. Thus, once the key to selecting the bath and the process for the coating is explained, it will be obvious to others skilled in the art just how to prepare additional baths for coating beryllium metal falling within the scope of my teaching.

The objects, features, characteristics, and advantages of the processes of my invention will be better appreciated from the following specific description in which the single figure is a pictorial representation of the physical components and arrangement necessary for accomplishing the coating process of my invention.

As pointed out above, various coating processes are available for beryllium metal. For example, a number of anodizing baths are capable of turning beryllium black. However, the baths do not produce coatings to which commercial high strength adhesives such as epoxy bond well. The conventional bath for blackening the exterior of beryllium metal is a chromic-acid/nitric-acid solution which may contain as much as 70° Baumé nitric acid (concentrated) and various other additives. The coating produced is black, but slick and uneven. The epoxy adhesives used in commercial bonding processes do not adhere well to the coat due to its slickness. The coating does adhere well to the beryllium metal which it protects.

However, in thin layers it is not sufficiently dielectric. Further, in thick layers the coating is quite uneven. In order to provide appropriate overall protection of the beryllium metal, the coating must be made so thick that general dimensions of the material are changed. This is due to the fact that these coatings build up to cover the surface of the metal.

In view of the inadequacy of the available anodizing baths for beryllium, experiments were conducted in the hope of discovering a bath which would provide the desired characteristics. It should be especially noted that a commercial sodium hydroxide bath was tried but proved incapable of producing the desired characteristics. A boric acid bath was also tried but appeared unsuccessful though indications were that the coating produced was slightly resistive; an ammeter used in circuit with a source of DC power showed a definite current drop as the coating formed. However, the coating produced was white and powder-like.

In view of the fact that the boric acid bath showed some possibility of producing at least one of the desired characteristics, an attempt was made to get more boric acid into the bath solution. To this end, sodium hydroxide (which had previously proved unsuccessful) was added. When the solution was at a point in which four gram-moles of boric acid were mixed with three gram-moles of sodium hydroxide in a liter of water, a heavy blue-white-gray coating was produced. The coating was quite dielectric and would not pass current detectable to my instruments. This was the first experimental success.

However, the coating abraded quite easily and had the wrong color for the planned use. Postulating that beryllium oxide formed by the anodization lent the gray to the coating, the sodium hydroxide concentration was increased and the boric acid concentration was decreased. This lessened the borate ion in solution and increased the beryllium oxide in the coating. When the concentration of the bath reached four gram-moles of sodium hydroxide and three gram-moles of boric acid, the coating turned black. This was the second success in the experiments. Thereafter, I found that by lowering the boric acid content of the solution a thinner film was possible. After considering the bath content, I decided to use sodium borate instead of boric acid and to adjust the solution to give different pH concentrations. This arrangement proved the key to success in anodizing beryllium metal to obtain the desired properties.

In each case, it was determined that a coating formed on the beryllium metal. However, the properties of the coating varied depending on the pH and pOH of the solution. For example, the coating which had formed when an excess of boric acid was included in solution, though dielectric, was white, thick, and non-adherent whereas the coating which formed when an excess of sodium hydroxide was included in the solution was dielectric, black, thin, and adherent. Thus, the characteristics of the coating clearly depended on the particular percentages of the acid and base used in the solution. After some experimenting, it was determined that the solution best adapted to produce the characteristics desired was one in which all acid was neutralized and excess hydroxyl ions were present. For example, a neutral solution of sodium borate to which was added sodium hydroxide, from a relatively minor amount to a saturated solution, would prove most useful. The various experiments demonstrated, however, that with different concentrations of sodium hydroxide or boric acid, with different initial voltages, with different temperature controls, and so on, the bondability of the coating could be varied, its color and hardness could be changed, and its other properties could be operated upon almost as desired.

In brief, the process of this invention amounts to an electrochemical formation of an oxide film of beryllium through the combination of ions from the bath solution with the beryllium metal anode. In the figure, a direct

current source is provided for biasing the beryllium metal anode to a positive potential. The other terminal of the biasing source is connected to another electrode to define a cathode. In a particular embodiment, the cathode is the stainless steel tank used to hold the bath solution. When current is passed through the bath solution shown in the tank of the figure, the coating immediately begins to form. An initial voltage as low as two volts may be used; how-

example, beryllium oxide is normally considered to be a white material. However, I have been able to form a blue coating, a dark grey or black coating, a tan coating, and a coating of other colors. I feel that the amounts of boron in the coating and other compounds of both beryllium and boron are present and affect the characteristics. The following tables list various properties of the coatings formed for particular solutions used:

TABLE I.—TEMPERATURE ADJUSTMENTS OF BATH SOLUTION  
[Ratio: Boric Acid 3/Sodium Hydroxide 3.5]

| Temp., ° F. | V <sub>1</sub> | V <sub>2</sub> | A <sub>1</sub> | A <sub>2</sub> | T <sub>1</sub> | T <sub>2</sub> | T <sub>3</sub>    | A    | ASF   | V.B. | Color        |
|-------------|----------------|----------------|----------------|----------------|----------------|----------------|-------------------|------|-------|------|--------------|
| 80.....     | 7.0            | 14.5           | 2.6            | 0.12           | .2506          | .2506          | .1>T <sub>3</sub> | 3.97 | 4.32  | 0    | Light Gray.  |
| 90.....     | 7.0            | 14.0           | 2.8            | 0.13           | .2500          | .2501          | .1                | 4.23 | 4.46  | 0    | Do.          |
| 100.....    | 7.0            | 13.8           | 2.9            | 0.195          | .2502          | .2503          | .1                | 3.75 | 7.49  | 0    | Do.          |
| 110.....    | 7.0            | 14.2           | 3.0            | 0.137          | .2502          | .2502          | .1>T <sub>3</sub> | 4.48 | 4.32  | 0    | Do.          |
| 120.....    | 7.0            | 14.5           | 4.0            | 0.250          | .2500          | .2500          | .1>T <sub>3</sub> | 4.72 | 7.63  | 0    | Light Brown. |
| 130.....    | 7.0            | 14.5           | 4.0            | 0.200          | .2502          | .2503          | .1                | 3.99 | 7.2   | 0    | Dark Brown.  |
| 140.....    | 7.0            | 16.0           | 5.8            | 0.260          | .2495          | .2495          | .1>T <sub>3</sub> | 3.78 | 8.78  | 0    | Do.          |
| 150.....    | 7.0            | 15.0           | 5.0            | 0.310          | .2502          | .2503          | .1                | 4.15 | 10.66 | 0    | Do.          |

V<sub>1</sub>=Initial voltage.  
V<sub>2</sub>=Final voltage.

T<sub>2</sub>=Thickness of coated sample.  
T<sub>3</sub>=Thickness of coating in mils.

A<sub>1</sub>=Initial amperage.  
A<sub>2</sub>=Final amperage.

A=Area in square inches.

T<sub>1</sub>=Thickness of bare sample.

V.B.=Voltage breakdown.

ASF=Amperes per square foot.

TABLE II.—TEMPERATURE ADJUSTMENTS OF BATH SOLUTION  
[Ratio: Boric Acid 3/Sodium Hydroxide 3.75]

| Temp., ° F. | V <sub>1</sub> | V <sub>2</sub> | A <sub>1</sub> | A <sub>2</sub> | T <sub>1</sub> | T <sub>2</sub> | T <sub>3</sub>    | A    | ASF  | V.B. | Color             |
|-------------|----------------|----------------|----------------|----------------|----------------|----------------|-------------------|------|------|------|-------------------|
| 80.....     | 7.0            | 13.7           | 3.2            | .245           | .2502          | .2503          | .1                | 3.87 | 9.07 | 0    | Tan.              |
| 90.....     | 7.0            | 14.5           | 4.8            | .455           | .2496          | .2497          | .1                | 4.51 | 15.6 | 0    | Dark Tan.         |
| 100.....    | 7.0            | 14.0           | 4.0            | .305           | .2488          | .2488          | .1>T <sub>3</sub> | 3.2  | 13.7 | 0    | Golden Brown.     |
| 110.....    | 7.0            | 13.5           | 4.5            | .620           | .2493          | .2493          | .1>T <sub>3</sub> | 4.03 | 22.2 | 0    | Black Violet.     |
| 120.....    | 7.0            | 14.5           | 5.6            | .720           | .2429          | .2429          | .1>T <sub>3</sub> | 4.03 | 25.6 | 0    | Metallic Blue.    |
| 130.....    | 7.0            | 13.7           | 6.0            | 1.120          | .2459          | .2459          | .1>T <sub>3</sub> | 4.28 | 37.6 | 0    | Olive Drab.       |
| 140.....    | 7.0            | 13.8           | 6.0            | 1.1            | .2464          | .2464          | .1>T <sub>3</sub> | 3.56 | 44.5 | 0    | Iridescent Brown. |
| 150.....    | 7.0            | 13.0           | 6.9            | 2.2            | .2491          | .2492          | .1                | 4.21 | 75.3 | 0    | Bluish Black.     |

V<sub>1</sub>=Initial voltage.

T<sub>2</sub>=Thickness of coated sample.

V<sub>2</sub>=Final voltage.

T<sub>3</sub>=Thickness of coating in mils.

A<sub>1</sub>=Initial amperage.

A=Area in square inches.

A<sub>2</sub>=Final amperage.

V.B.=Voltage breakdown.

T<sub>1</sub>=Thickness of bare sample.

ASF=Amperes per square foot.

TABLE III.—INITIAL VOLTAGE ADJUSTMENTS OF BATH SOLUTION  
[Ratio: Boric Acid 3/Sodium Hydroxide 3.75]

| Temp., ° F. | V <sub>1</sub> | V <sub>2</sub> | A <sub>1</sub> | A <sub>2</sub> | T <sub>1</sub> | T <sub>2</sub> | T <sub>3</sub> | A    | ASF  | V.B. | Color                 |
|-------------|----------------|----------------|----------------|----------------|----------------|----------------|----------------|------|------|------|-----------------------|
| 120.....    | 2.0            | 4.2            | .290           | .080           | .2501          | .2501          | -----          | 3.97 | 10.5 | 0    | Light Gray.           |
| 120.....    | 4.0            | 5.0            | 1.0            | .750           | .2496          | .2496          | -----          | 4.23 | 34.0 | 0    | Gray.                 |
| 120.....    | 6.0            | 8.5            | 3.2            | 1.8            | .2500          | .2500          | -----          | 3.75 | 29.9 | 0    | Black<br>(periphery). |
| 120.....    | 8.0            | 16.0           | 6.6            | .8             | .2500          | .2500          | -----          | 4.48 | 62.0 | 0    | Dark Brown.           |

Columns have the same meanings as in the above tables.

ever, better properties will be obtained where the initial voltage is maintained at five or six volts. However, higher voltages may be used. In a particular embodiment, the temperature of the bath need only be maintained between 70° and 180° Fahrenheit. Current is applied until the required thickness of coating is formed (e.g., from fifteen minutes—one hour). In one exemplary bath, a neutral solution of sodium borate is mixed with a small amount of sodium hydroxide to provide an excess of hydroxyl ions. An especially useful solution contains sodium borate and sodium hydroxide in a ratio of 2.69 gram-moles to 0.77 gram-moles. As a potential is applied, oxygen is produced at the anodes, forming an oxide coating on the beryllium metal. By controlling the temperature of the bath (through the temperature control shown on the figure), the duration of the process, the initial voltage applied to the voltage control, the pH of the solution, and by selecting an appropriate surface treatment for the beryllium metal, an infinite range of colors, thicknesses, surfaces, and conductivity properties may be obtained.

I believe the coating actually comprises beryllium oxide held in a covalent bond with boron. The structure of the beryllium is such that it may form a number of different covalent bonds when different electrons are shared with oxygen thereby providing the different characteristics. For

In a preferred process in accordance with the invention, the bath comprises sodium borate having a consistency of 177 grams per liter and sodium hydroxide having a consistency of 30 grams per liter. The bath is used at an operational temperature of 100° to 120° Fahrenheit. An initial voltage of six volts is applied. The process continues for a period of one hour. No particular preparation is necessary for this preferred bath though normally one of the chemicals is dissolved in solution and the bath brought to temperature before the other is added.

The surface of the material is cleaned in a manner to provide the desired final finish. In this regard it should be noted that no special cleaning techniques are required for this bath. This is in contrast to the cleaning techniques necessary for anodizing aluminum in the standard chromic acid bath.

The material to be anodized is placed in the bath solution as the anode. The electrical connection to this material is normally insulated from the bath solution to prevent an inappropriate anodizing from occurring at the connection itself. The conductor to the anode may be coated with a plastic material which is unaffected by the anodizing bath; or an electrical connection of the same material, beryllium, may be used. The particular operation is substantially insensitive to minor variations in

parameters and produces a coating which is black, dielectric (measures 300-500K ohms resistance), thin, bondable, and has a selectable surface and dimensions.

Certain of these characteristics are of especial importance. For example, the lack of special cleaning techniques eliminates one of the very expensive steps of most anodizing processes. It also allows the surface to be prepared as one desires for the final coating. This results because the coating, though dielectric, may be made so thin that the dimensions remain substantially the same. A typical dimensional change is 0.0002 inch. Thus, if a very smooth mirror-like surface is prepared on the beryllium metal, the same surface will appear on the final coating. On the other hand, if a stippled surface is prepared, a stippled surface will result for the coating. Also of especial importance with regard to the thickness and finish of the coating is the fact that dimensions need not be programmed for the coating to allow corrections for add on during the process. The coating is actually formed with the surface beryllium and is so thin that essentially the same dimensions and surface remain after the coating as those of the original material. The same surface remains though its constituency has changed. This is especially important in manufacturing precise instruments.

The multi-colored aspect of the coating allows a selection for decorative, industrial, or other purposes. For example, the original black coating was chosen because a heat emissive exterior was desired for the particular instrument. On the other hand, it might be desirable to identify certain portions of a complex process by the color of the materials used. With this bath, identifications could be accomplished by color. It should be particularly noted that the coloring is accomplished in the bath without the necessity of a dyeing process, as is usual in aluminum anodizing. Thus, another step is eliminated from conventional processes. Further, the entire coating is of the selected color rather than just the surface portion so that the abrasion of the material is not so likely to cause flaws in the color as with aluminum anodized material.

The wide temperature range by which it is possible to reach substantially the same results is especially valuable in providing a process which may be run by industrial workers. This advantage obviously adds to the economies of the proposed process. On the other hand, the low power and the short time necessary for the anodizing materially reduce processing costs.

As pointed out before, the conductivity of the coating may be varied as desired. In the particular instrument for which the coating was originally prepared a dielectric coating was desired. Such a dielectric coating is especially useful in preventing electrical shorts and leakage in precision instruments and substantially eliminates galvanic corrosion which may tend to effect rapid deterioration of precision instruments using some prior art coatings.

The bondability of the surface produced by the preferred process is also especially desirable. The prior art techniques for producing a black coating on beryllium evidently were not gauged with modern production processes

in mind, and the slick coating formed by some of the prior art techniques limited the techniques by which beryllium parts could be made to adhere to other elements. With commercial epoxy adhesives designated FA8 and LCA 4/9, a minimum block shear strength of 6100 p.s.i. was obtained.

The coating may be made both abrasion and corrosion resistant. For example, when subjected to a 5% salt water solution and to like vapors, the coating showed no effect after 120 hours though beryllium metal was severely etched after the same period.

Having shown the techniques for selecting the various combinations used in the bath and the different controlling elements in the process, those skilled in the art will be able to devise numerous other baths, processes, and coatings. For these reasons, the invention is to be considered as restricted only within the scope of the appended claims.

#### What is claimed is:

1. A method of coating beryllium comprising the steps of immersing a piece of beryllium in an aqueous alkaline bath having a free hydroxyl ions and borate ions, placing a potential between said piece and a second terminal sufficient to generate a current in said bath wherein said piece is anodic, and anodizing said piece to produce a coating thereon.
2. The product produced by the process of claim 1.
3. A process of anodizing beryllium comprising the steps of preparing a desired surface on the beryllium metal by a selected cleaning technique, immersing the beryllium metal in an aqueous alkaline bath of an alkali metal borate solution containing free hydroxyl ions, connecting a source of potential between the beryllium metal as anode and a cathode, and passing current through the electrolyte bath by means of the source for a selected time.
4. A method for selectively coloring beryllium comprising the steps of preparing an aqueous alkaline bath comprising sodium hydroxide and boric acid having free hydroxyl ions, immersing the beryllium in the bath, connecting the beryllium to a positive terminal of an electrical source, applying a selected voltage between the beryllium and another point in the bath sufficient to pass current through the bath, and maintaining the current for a selected period.

#### References Cited

##### UNITED STATES PATENTS

|           |         |          |           |
|-----------|---------|----------|-----------|
| 2,373,273 | 4/1945  | Sziklai. |           |
| 2,871,425 | 1/1959  | Burnham  | 204-56 XR |
| 3,180,807 | 4/1965  | Quinn    | 204-56 XR |
| 3,276,974 | 10/1966 | Tyson    | 204-56 XR |

##### FOREIGN PATENTS

|         |        |                |
|---------|--------|----------------|
| 813,994 | 5/1959 | Great Britain. |
|---------|--------|----------------|

55 HOWARD S. WILLIAMS, *Primary Examiner.*

ROBERT K. MIHALEK, *Examiner.*

G. KAPLAN, *Assistant Examiner.*